

Dec. 29, 1936.

M. C. TEVES

2,066,081

PHOTOTUBE

Filed March 13, 1935

*Fig. 1*



*Fig. 2*



INVENTOR.  
MARTEN CORNELIS TEVES

BY

*Charles M. Clair*  
ATTORNEY.

## UNITED STATES PATENT OFFICE

2,066,081

## PHOTOTUBE

Marten Cornelis Teves, Eindhoven, Netherlands,  
assignor to Radio Corporation of America, a  
corporation of Delaware

Application March 13, 1935, Serial No. 10,764  
In Germany March 26, 1934

3 Claims. (Cl. 250—27.5)

My invention relates to light sensitive electron discharge devices, more particularly to improvements in photo-cathodes and the method of manufacturing the same.

5 In the manufacture of photo-tubes having photo-electric electrodes or photo-cathodes which have a high electron emitting capacity, it is conventional practice to deposit a metal layer, usually of silver, on the inside wall of 10 the tube envelope and to then superficially or entirely oxidize this layer and subject it to the action of an electropositive metal, for example, an alkali or alkaline earth metal. The oxidation of the silver metal layer is usually effected by 15 heating the metal in an atmosphere containing oxygen or by means of an electric discharge in such an atmosphere.

It has been found that this oxidation method introduces a number of difficulties. The oxidation by electrical means for example is limited 20 substantially to the oxidation of silver layers. When other metals, for example, copper and nickel are used, the results are often unsatisfactory. When it is desired entirely to oxidize the 25 metal layer, and if it is deposited on an insulating base, for example, glass, the oxidation takes place irregularly and not to the same depth throughout the metal layer. Because of this, parts of the layer which are not oxidized are 30 separated by parts of the layer which have been completely converted into oxide, the result being that current passes thru the electrode with difficulty or not at all. While further oxidation is 35 not impossible, it is nevertheless considerably hampered. If the metal layer which is to be entirely transformed into a metal oxide, is applied to a metal base, the irregular oxidation of the metal layer results in a layer which is not completely 40 oxidized or, in oxidizing the base at numerous points. This difficulty is encountered, for example, when a thin silver layer applied to a copper or nickel layer is to be oxidized. The copper or nickel oxide introduces difficulties when the electropositive or alkaline earth metal acts on the 45 silver oxide. Such difficulties also occur when the metal layer is oxidized by heating in an atmosphere containing oxygen.

The object of my invention is to provide an improved method of manufacturing a photo-cathode having a uniform structure and which can be provided on either an insulating or conducting base.

According to my invention the metal from 50 which the oxide layer is formed is supported within the tube envelope out of contact with the

base on which the oxide layer is to be formed. A discharge in an atmosphere containing oxygen is established within the discharge tube between the metal and another electrode, the metal serving as a cathode. The position of this metal as well as the current strength are so chosen that a layer of oxide of the metal deposits on the base. In this way a uniformly oxidized layer is obtained. My invention is particularly suitable for manufacturing photo-electric electrodes which must be transparent to light and in which the metal oxide layer must be formed on glass or a similar material transparent to light. The electrodes manufactured according to my invention can be rendered emissive not only by light but also 15 by other means, for example, by ion or electron bombardment causing secondary emission.

The novel features which I believe to be characteristic of my invention are set forth with particularity in the appended claims, but the invention itself will best be understood by reference to 20 the following description taken in connection with the accompanying drawing in which:

Figure 1 is a vertical section of a light sensitive electron discharge device by means of which my invention may be practiced.

Figure 2 is a perspective of a light sensitive electron discharge device of different construction by means of which my invention may be practiced.

In Figure 1 a photo-electric tube having a glass envelope 1, is provided with a stem 2 to which is secured a metal rod 4 consisting, for example, of molybdenum, and at the end of which is provided a block 5 of silver. The rod 4 is surrounded by an insulating tube 3. The stem also carries a short rod 6 which like the rod 4 is connected to a current supply wire. A conductor 7 bearing on the inner side of the wall of the tube envelope is sealed into the wall opposite the stem 2.

After the envelope 1 has been exhausted, a small 40 quantity of oxygen, for example, at a pressure of about 1 mm of mercury is introduced into the envelope, and an electric discharge established between the silver block 5 (which acts as a cathode) and the rod 6 (which acts as an anode). 45 The current strength is so chosen that the silver block 5 disintegrates and a silver oxide layer 8 deposits on the wall of the envelope. In some cases excellent results have been obtained with current intensities of a few milli-amperes for example. It has been found that the silver oxide 50 layer is very regular and that the thickness of the layer can be regulated within fine limits by maintaining the discharge for a longer or shorter period of time.

After the silver oxide layer 8 has been formed, the remaining oxygen is removed from the envelope and caesium or another alkali metal is introduced and made to react with the silver oxide in a well-known manner, for example, as described in U. S. patent 1,901,578 to Bainbridge. The silver oxide is reduced, forming a layer consisting of a mixture of silver particles, caesium particles and caesium oxide particles, on which 10 is deposited a thin caesium layer. If desired, the excess of caesium may either be removed from the envelope or bound therein in a conventional manner.

The wire 7 sealed into the wall constitutes 15 the electric conductor for the photo-electric electrode or photo-cathode thus formed. The cathode is made thin enough to be transparent to light so that the light rays impinging on the outside of the envelope can pass thru to the 20 inner side of the cathode. Therefore, it is not necessary to provide a window in the cathode. To avoid the formation of a conductive layer on the stem, it may be shielded by means of a 25 screen in the course of manufacture.

25 In the modification shown in Figure 2, the photo-electric electrode of the tube is formed on the semi-cylindrical body or electrode 9 which may consist of copper and is supported from the stem 2. This stem also supports the electrode 30 10 consisting of a silvered molybdenum rod. After exhaustion of the tube oxygen is introduced and a discharge is established between the body 9, which acts as an anode, and the rod 10, which 35 acts as a cathode, the current strength used having such a value that the hollow side of the body 9 is coated with a silver oxide layer which is subsequently subjected in the manner set out above to the action of the electropositive metal.

The electrode 9 which receives a positive voltage with respect to the electrode 10 when the 40 silver oxide layer is formed has with a normal use of the tube a negative potential with respect to the electrode 10, which acts as the anode.

While I have indicated the preferred embodiments of my invention of which I am now aware and have also indicated only one specific application for which my invention may be employed, it will be apparent that my invention is by no means limited to the exact forms illustrated or 45 50 the use indicated, but that many variations may be made in the particular structure used and the purpose for which it is employed without departing from the scope of my invention as set forth in the appended claims.

55 What I claim as new is:—

1. The method of manufacturing a photo-cathode for a light sensitive electron discharge de-

vice having an envelope in which a metal oxide layer is to be formed and subjected to the action of an electropositive metal, which includes positioning the metal from which the oxide layer is to be formed within the envelope out of contact 5 with a base within the envelope on which the metal oxide layer is to be formed, introducing an atmosphere containing oxygen within said envelope, establishing a controlled electric discharge between said metal as a cathode and another 10 electrode as an anode within the envelope, so that a layer of the oxide of said metal is deposited on said base, removing the atmosphere containing oxygen from the interior of the envelope and introducing an alkaline metal within 15 the envelope to reduce the metal oxide to form a light sensitive electrode on the interior of the envelope.

2. The method of manufacturing a photo-cathode in a light sensitive electron discharge device 20 having an envelope of glass on which a metal oxide layer is to be formed and subjected to the action of an electropositive metal, including 25 positioning within the envelope and out of contact with the envelope the metal from which the oxide layer is to be formed, introducing within the envelope and atmosphere containing oxygen, establishing a discharge between said metal and an auxiliary electrode within said 30 envelope, said metal serving as a cathode and said auxiliary electrode as an anode during said discharge, and controlling the strength of the discharge so that a metal oxide layer thin enough to be transparent to light is formed on the inside 35 of the envelope, removing the atmosphere containing oxygen from the interior of the envelope and introducing an alkaline metal within the envelope to reduce the metal oxide to form a light sensitive electrode on the interior of the envelope. 40

3. The method of manufacturing a photo-cathode in a light sensitive electron discharge device having an envelope containing a pair of parallel electrodes, one of the electrodes including a 45 silvered molybdenum rod and the other a semi-cylindrical copper body, including exhausting the envelope, introducing oxygen into said envelope, establishing a discharge between the electrodes, the silvered molybdenum rod acting as a cathode and the copper body as an anode during the discharge to form a silver oxide layer on the copper body, exhausting said oxygen from said envelope and subjecting the resulting oxide layer on said copper body to the action of an electropositive metal to form a light sensitive photo-cathode. 50 55

MARTEN CORNELIS TEVES.